

Dec. 5, 1933.

H. J. BILLINGS

1,937,680

MOLDABLE MATERIAL

Filed Nov. 6, 1929



Inventor:  
Howard J. Billings.  
By Roberts, Cushman & Woodbury  
his Attorneys.

## UNITED STATES PATENT OFFICE

1,937,680

## MOLDABLE MATERIAL

Howard James Billings, South Acton, Mass., assignor to Arthur D. Little, Incorporated, Cambridge, Mass., a corporation of Massachusetts

Application November 6, 1929. Serial No. 405,145

20 Claims. (Cl. 154—2)

This invention relates to a moldable material having the property of combining in a plied construction under the influence of heat and pressure and to the method for forming and treating such material.

The preferred components of such material are briefly paper pulp and a binder comprising hardwood pitch suitably treated with a gum, the fibers of the pulp and the particles of binder intimately distributed throughout the body, which is in sheet form, but the fibers and particles are discrete and not adhesively associated until heat and pressure is applied.

An article formed from such material is moisture resistant and dielectric and is applicable to many uses wherever such qualities are desirable. Such an article is of particular value as a core or backing for a sound record of the type set forth in my copending application Serial No. 378, 20 893, filed July 17, 1929, in place of the one therein described which consisted of laminae of combining and filling sheets alternately arranged.

The combining sheets for the core or backing of the sound record set forth in that application contained shellac as a binder and hence are more expensive to manufacture than are sheets embodying this invention. Moreover, since a core embodying this invention consists of laminae, each comprising fibers and a binder, it is more effectively moisture resistant than the core disclosed in my prior application, a sound record embodying this invention will be substantially unaffected by moisture and other climatic conditions.

One object of this invention is to provide a moldable material having the properties and structure hereinafter set forth. Another object of this invention is to provide a sound record similar in characteristics to that set forth in my copending application but having a core which is cheaper than that disclosed therein and which has a greater resistance to warping. While certain of these characteristics as well as the structure and the method of making the sound record will be set forth herein, reference may be made to such application for a fuller disclosure thereof.

Other objects will appear from a consideration of the following specification and of the drawing which forms a part thereof and in which

Fig. 1 is a diagrammatic view of a sound record blank embodying this invention, the various laminae being shown as separated for the purpose of clarity;

Figs. 2 and 3 are enlarged sectional views of a portion of such sound record blank illustrating

the relation of the laminae before and after the sound grooves have been formed therein; and

Fig. 4 is a view illustrating diagrammatically one way of making upon a paper machine a sound record embodying this invention.

Referring to the drawing, the sound record 10 comprises two record sheets 11 which are in the usual way, provided on their exposed faces with playing surfaces and a core 12 here shown as consisting of two laminae or sheets made in the manner described hereinbelow. For the purpose of illustrating one application of this invention I have elected to show the core as comprised of two such laminae but it will be understood that the number thereof may be varied as desired.

The moldable material is made in sheet form on a paper machine from a composition consisting of fibrous material and a binder. The fibrous material and binder vary in proportions depending upon the type of fibrous material used, but it has been found that the composition should contain at least sixty per cent. of binder in order to insure a material having the necessary cohesive and adhesive qualities.

The following formula has been found to give 80 satisfactory results:

| No. 1                  |    | Pounds |
|------------------------|----|--------|
| Fibrous material 32.8% |    |        |
| Kraft pulp             | 20 | 85     |
| Unbleached sulfite     | 5  |        |
| Ground wood            | 14 |        |
| Binder 67.2%           |    |        |
| Hardwood pitch         | 36 |        |
| Ternati gum            | 36 |        |
| Rosin                  | 8  | 90     |

If desired the unbleached sulfite and ground wood may be replaced by nineteen pounds of old newspaper. A coloring material, such as for example carbon black, may be added to the mixture and with the formula above given three and one-half pounds should be used. Changes in material and in proportions may be made and I am not limited to the above formula which is set forth merely as a preferred illustration.

The fibrous material and binder are processed into a pulp in the following manner: The fibrous materials given with the exception of ten pounds of the kraft pulp is treated with six gallons of water and then kneaded with the binder under the influence of heat to effect a thorough distribution of the binder over the wet fibers. This is preferably accomplished in a kneading machine of the type in which kneading blades, rotating inwardly, work the mass of binder and fibrous material under a superimposed mechanical pres-

sure exerted by a ram fitting into the charging neck of the machine. The whole mass is then broken down to a watery pulp containing intimately distributed discrete particles of fiber and binder, by the addition of twelve gallons of hot water. The watery pulp is finally fibrated in a paper mill beater, the kraft pulp previously withheld being added at this time and is now suitable for forming into sheets on a paper machine in the usual manner.

The sheets of moldable material so made must contain a binder which, under the application of heat and pressure as in a press, becomes sufficiently fluid to coat the fibers and prevent the absorption of moisture from without and sufficiently cohesive so that the laminae are firmly united in a solid mass, the line of demarcation between the laminae being practically eradicated. This requirement necessitates a consideration of the physical characteristics of the binders that might be used, namely, the softening point (determined by the ball-and-ring method in plastics which have no sharp melting point) and the susceptibility factor.

25 The softening points of the hardwood pitch alone and of the binder set forth in Formula No. 1, as determined by the ball-and-ring method, are 180° F. and 210° F. The comparative susceptibility of these two materials is shown by penetration tests at various temperatures as follows:

| Temper-<br>ature | Hardwood<br>pitch | Binder |
|------------------|-------------------|--------|
| 77° F.....       | 0                 | 0      |
| 115° F.....      | 8                 | 2      |
| 150° F.....      | 45                | 10     |
| 175° F.....      | 81                | 20     |

35 The susceptibility factor, as ordinarily understood in this connection, is a numerical expression which indicates the response of a plastic substance to temperature changes, a material with a high susceptibility factor changing from the solid to the fluid state within a relatively short temperature range and a material with a low susceptibility factor changing from the solid to the fluid state within a relatively long temperature range.

A sheet made in accordance with this invention must therefore contain a binder which not only has the proper softening point but also has a low susceptibility factor so that it will become increasingly plastic, without actually being fluid, in the presence of the heat to which the sheet will be subjected. Such a binder will possess only the necessary amount of flow in the presence of heat and pressure to cement the laminae together and to hold them united after the heat and pressure are removed, and also to ensure a complete coating of the fibers, thus rendering them reasonably impervious to climatic actions of moisture and temperature.

While shellac is the most satisfactory material for this purpose, it is too high in price to be used as a binder, particularly when it must be the sole binder used. Hardwood pitch when fluxed with certain gums having a low susceptibility factor, such as a manila gum (for example, ternati gum or manila nubs), I have found to be satisfactory for the purpose described as a substitute for shellac. Copal gums or other gums having a low susceptibility factor might be used with the hardwood pitch if desired.

The hardwood pitch alone has too low a softening point and hence is too fluid at the molding

temperatures used in carrying out this invention. If a core of hardwood pitch alone were embodied in a sound record of the type set forth in my co-pending application, it would, due to this fluidity, flow through the record sheets to the playing surfaces, which would thereby be impaired and rendered more or less wholly unsuited for playing. The manila gums, on the other hand, have a low susceptibility factor which causes them to become increasingly plastic, without actually melting, through a relatively long range of temperature in the presence of the required heat but have too high a softening point. The mixture, however, of hardwood pitch and a manila gum, has the desired softening point which is above that of the pitch and below that of the manila gum and yet has susceptibility characteristics of the kind possessed by the manila gum. For this reason I have found the above-recited formula to be satisfactory.

I make a final adjustment of the softening point to the desired level by adding to the manila gum-hardwood pitch mixture a small amount of rosin. I attribute no properties to this rosin other than the modification of the softening point and it is conceivable that other grades of hardwood pitch could be used which would require the addition of little or no rosin.

The mixture made in accordance with the above formula has therefore, due to the presence of the fibrous material, toughness and flexibility and, due to the presence of the binder, the faculty of flowing freely under the heat and pressure to which it is subjected and a low susceptibility factor.

50 In the manufacture of sound records and other articles the compound above described is used as a core having on each outer face a record sheet 11 into which the sound grooves are formed by the use of heat and pressure in a die in the usual manner. The record sheets may be composed as disclosed in my co-pending application or may have substantially the following formula:

| No. 2                  | Pounds                    |
|------------------------|---------------------------|
| Thermoplastic material | Shellac..... 64           |
|                        | Rosin..... 6              |
| Fibre                  | Kraft pulp..... 15        |
|                        | Unbleached sulfite..... 4 |
|                        | Ground wood..... 13       |
| Filler and color       | Clay..... 20              |
|                        | Carbon black..... 3 1/2   |

55 The various materials are treated in the manner above described with reference to the core material and formed into sheets. The formula may be modified in various ways both as to materials and proportions. Thus, in place of shellac and rosin, shellac alone may be used, or other resins or thermoplastics may be used, either alone or in combination, if suitable for a playing surface. Other fillers, as for example, graphite may be used in place of or in combination with the fillers above mentioned.

60 The sheets thus formed are provided with a coating consisting of a binder, an abrasive filler, a filler to give body and a pigment. This coating may be in accordance with Formula No. 3 of my co-pending application and may be applied either by the dry or the wet method therein set forth. In the dry method the powdered composition is dusted upon the sheets and caused to adhere thereto by passing the sheets through an oven so that the powder is incipiently fused. In the wet method the composition is ground in water 150

forming a paint which is applied as a liquid to the sheets by means of a brush or in any desired manner and sets upon drying.

One way of making a sound record is to cut 5 from the core and record sheets discs which are assembled as shown in Fig. 1 of the drawing after having been thoroughly dried to expel any free moisture therein. The assembled discs are then placed in a press between stampers bearing the sound grooves. These stampers are each 10 mounted on a platen or die through which steam or water may be circulated to raise or lower the temperature of the material in the press. The press is then closed to bring the stampers into 15 contact with the record sheets, and held in that position for twenty seconds without exerting the full pressure. During this period steam is circulated through the platens or dies under a pressure of approximately eighty to one hundred pounds 20 pressure per square inch. Pressure is then applied for a period of fifteen seconds (thirty tons in case of a record blank ten inches in diameter) while the circulation of the steam continues. The steam is next shut off and cold water circulated 25 until the record blank is cold whereupon the cold water is shut off, the press opened and the record removed.

The heat applied at the first stage of the above 30 operation causes the moldable material forming the various sheets to become plastic so that under the influence of the heat and pressure at the following stage the binders will flow, coating the fibers and combining the various sheets into a unitary structure. In this connection it will be 35 noted that the softening point and susceptibility factor of the binder in the core sheets has been so set that the binder therein will not exude to any appreciable extent into the record sheets and thus impair the playing surface, but will however unite the core sheets to the record sheets. In the record blank made according to the invention disclosed in my copending application plain 40 binder free filler sheets were inserted between the combining sheets of the core and the record sheets; this however is not necessary according to the present invention by reason of the materials used in the formation of the core sheets. The binder of the core sheets has a somewhat higher 45 softening point than the binder of the record sheets but has a low susceptibility factor so that the binder of the core sheets will not penetrate the record sheets to the playing surfaces thereof.

The edges of records made by my process may be smoothed as desired by simple abrasion. No 50 special type of apparatus is necessary for this purpose and there is no need for much precaution against breaking the records as they are very resistant to shock. When the records are so abraded, or when their edges are cut with a knife, it 55 will be observed that the record acts as a unitary structure rather than as a series of laminations; the lamellar structure possessed by the parts before being united in the press having substantially disappeared.

The grooves in the playing surface are produced and formed in the manner and of the structure set forth in detail in my copending application as will appear from Fig. 3 of the drawing. The sound records so produced like 60 those disclosed in my copending application are much lighter than the sound records commercially manufactured at the present time, are tough and not easily frangible. They can therefore be economically transported or sent through 65 the mails since the necessity of expensive pack-

ing does not exist. One of these records may be dropped upon the floor without injury to the playing surface, may be bent, snapped or subjected to shock and will retain its original condition without developing any surface cracks or hair lines in the playing surfaces which would have a deleterious effect upon its use as a sound record.

A record, ten inches in diameter, comprising two record sheets and two core sheets weighs between three and one-half and four ounces, whereas other well known records of the same diameter, now on the market, weigh from seven to seven and a half ounces each. The record sheets used are between twenty-three and twenty-four points thick while the core sheets are approximately twenty-eight and a half points thick making a total thickness of about one-tenth of an inch. While these dimensions have produced records which have proven to be very satisfactory, it is, of course obvious that they may be altered as desired and the number of core sheets increased without departing from the spirit and scope of this invention.

Instead of making the core and record sheets separately as in the method above described I 100 have found it desirable to unite part or all of the record and core sheets directly upon a paper machine of the multicylinder type. For instance a machine having two cylinders may be used as suggested in Fig. 4. The core sheet 15 and the 105 record sheet 16 are united at the rollers 17 in the usual way so that the result is a two-ply sheet, one ply being a core sheet made according to Formula No. 1 with a binder of hardwood pitch and manila gum and the other ply being a record 110 sheet made according to Formula No. 2 with a binder of shellac and rosin or other thermoplastic material capable of providing a suitable playing surface. Discs are then cut from the two-ply sheet dried, assembled with the surfaces of 115 the record sheets exposed and treated in a press in substantially the manner described above. The number of plies may be varied by using a paper machine having more cylinders. Thus I have found that a very satisfactory record can 120 be made by using a four cylinder machine to produce four ply sheets consisting of one record sheet 125 ply and three core sheet plies and assembling the discs cut therefrom to form an eight ply record.

The moldable material having a binder of hardwood pitch and manila gum may be subjected to heat and pressure with or without the moldable material having a binder of shellac and rosin to form poker chips, buttons, tiles, insulating panels 130 and like moldable articles which are required to be tough and can be made from laminated sheets. In all these articles the binders of the various laminae, under the molding heat and pressure, flow to coat the fibers therein and bind the 135 laminae in one unitary structure.

From the above description of the steps of making and molding this material it will be apparent that it responds to the molding step in a very different way from that in which paper saturated 140 with the above or any other binders would respond. This follows from the fact that in the formation of the sheets the fibers and particles of binder are intimately distributed through the mass but remain substantially independent and the fibers are felted in the presence of the binders under the application of the molding heat and pressure, whereas the fibers of a saturated sheet are of course already felted independently of the saturant and thus when the molding heat and 145 pressure is applied the fibers are not felted together.

pressure are applied the result is a hard frangible structure.

It will be noted that the treatment of the sheets of moldable material embodying this invention 5 includes the step of drying the sheets thoroughly before placing them in the press. Such treatment however does not require that the sheets be at any particular temperature at the time they are placed in the molding machine. Consequently 10 it is possible to employ a machine in which a plurality of articles may be molded simultaneously. Such would not be true if it were essential that the sheets be at a certain temperature at the initiation of the molding operation.

15 I claim:

1. Moldable material comprising fibrous material and a binder consisting of hardwood pitch and a gum having a low susceptibility factor, said binder constituting at least sixty per cent of the 20 moldable material.

2. Moldable material comprising fibrous material and binder consisting of hardwood pitch and manila gum, said binder constituting at least sixty per cent of the moldable material.

25 3. Moldable material comprising fibrous material and binder consisting of hardwood pitch and manila gum, said binder constituting at least sixty per cent of the moldable material, the fibers and particles of binder being intimately distributed through the material as discrete particles.

35 4. Moldable material comprising fibrous material and binder consisting of hardwood pitch and manila gum, said binder constituting at least sixty per cent of the moldable material, the binder being thoroughly distributed as particles over the surfaces of the individual fibers and being independent thereof.

5. A laminated sheet of moldable material one 40 lamina comprising fibers and a binder including shellac and another lamina comprising fibers and a binder including hardwood pitch.

45 6. A laminated sheet of moldable material one lamina comprising fibers and a binder including shellac and another lamina comprising fibers and a binder including a gum having a low susceptibility factor.

50 7. An article consisting of laminae of moldable material subjected to heat and pressure, the laminae comprising fibers and a binder including hardwood pitch and manila gum, said binder coating said fibers to prevent their exposure to moisture and uniting said laminae.

55 8. An article consisting of laminae of moldable material subjected to heat and pressure, each lamina comprising fibers and at least sixty per cent of binder, said binder including substantially equal quantities of hardwood pitch and manila gum coating said fibers to prevent their 60 exposure to moisture and uniting said laminae.

65 9. An article consisting of laminae of moldable material subjected to heat and pressure, each lamina comprising fibers and at least sixty per cent of binder, said binder coating said fibers to prevent their exposure to moisture and uniting said laminae.

70 10. A sound record consisting of lamination of moldable material the outer lamina comprising fibers and a binder of thermoplastic material suitable for a playing surface, and the inner laminae comprising fibers and a binder including 75 hardwood pitch and manila gum.

11. A sound record consisting of laminations of moldable material, the outer laminae comprising fibers and a binder of thermoplastic material

suitable for a playing surface and the inner laminae comprising fibers and a binder including substantially equal amounts of hardwood pitch and manila gum.

12. A sound record comprising record sheets having playing surfaces and a core consisting of laminae, each comprising fibers and a binder including a mixture of hardwood pitch and manila gum with a low susceptibility factor, said binder coating said fibers to prevent their exposure to moisture, uniting the laminae of the core and uniting the core to the record sheets.

13. A sound record comprising record sheets having playing surfaces and a core consisting of laminae, each comprising fibers and a binder including a hardwood pitch having a relatively low susceptibility factor, said binder coating said fibers to prevent their exposure to moisture, uniting the laminae of the core and uniting the core to the record sheets.

14. The method of treating moldable material which method consists in the following steps, making a sheet of moldable material comprising fibrous material and a binder consisting of hardwood pitch and a gum having a low susceptibility factor, the fibers and particles of binder being intimately distributed through the sheet as discrete particles and subjecting said sheet to heat and pressure whereby the binder is caused to flow, coating the fibers and exuding to the surface thereof.

15. The method of treating moldable material which method consists in the following steps, making a sheet of moldable material comprising fibrous material and a binder consisting of hardwood pitch and a gum having a low susceptibility factor, the fibers and particles of binder being intimately distributed through the sheet as discrete particles, cutting blanks from said sheet, assembling said blanks in layers and subjecting 115 said blanks to heat and pressure whereby the binder in the blanks is caused to flow, coating the fibers therein and uniting the layers into a unitary structure.

16. The method of molding a laminated sound record in a press, said record including outer laminae each of which comprises fibrous material and a thermoplastic binder, and inner laminae each of which comprises fibrous material and a binder consisting of hardwood pitch and a gum having a low susceptibility factor, which method includes as steps uniting an outer lamina and at least one inner lamina to form a multi-ply blank, assembling two such blanks with the inner laminae in contact and subjecting them to heat 125 and pressure sufficient to cause the binder in the laminae to flow and unite the blanks into a unitary structure.

17. A record blank consisting of laminations of moldable material, the outer lamina comprising fibers and a binder of thermoplastic material, the inner lamina comprising fibers in a felted structure and a binder and a playing surface including a binder on the outer lamina adapted to receive and retain record grooves, the binder of 135 the inner lamina having a higher melting point than the binder of the playing surface, said fibers and binder being intimately associated, and capable of flowing under heat and pressure.

18. A record blank consisting of laminations of 145 moldable material, the outer lamina comprising fibers and a binder including shellac and providing a playing surface adapted to receive and retain record grooves, and the inner lamina comprising fibers and a binder including a hardwood pitch 150

having a low susceptibility factor, said fibers and binder being intimately associated as discrete particles.

19. A record blank consisting of laminations of moldable material, the outer laminae comprising fibers and a binder of thermoplastic material and providing a playing surface adapted to receive and retain record grooves, and the inner laminae comprising fibers and a binder intimately associated as discrete particles, said binder including a gum having a low susceptibility factor and being present in an amount sufficient to coat said fibers and to unite the inner laminae with each other and also to the outer laminae when the record blank is subjected to heat and pressure.

20. A record blank consisting of laminations of moldable material, the outer laminae comprising fibers and a binder of thermoplastic material and providing a playing surface adapted to receive and retain record grooves, and the inner laminae comprising fibers and a binder intimately associated as discrete particles, said binder including a hardwood pitch having a low susceptibility factor and present in an amount sufficient to coat said fibers and to unite the inner laminae to each other and also to the outer laminae when the record blank is subjected to heat and pressure.

HOWARD JAMES BILLINGS.

20

90

25

95

30

100

35

105

40

110

45

115

50

120

55

125

60

130

65

135

70

140

80

85

90

95

100

105

110

115

120

125

130

135

140

145